

# UNITED STATES PATENT OFFICE.

LEWIS N. JONES, OF ELSMERE, DELAWARE.

## METHOD OF MAKING FIBER SHEETS.

1,110,140.

Specification of Letters Patent.

Patented Sept. 8, 1914.

No Drawing.

Application filed January 28, 1914. Serial No. 815,053.

To all whom it may concern:

Be it known that I, LEWIS N. JONES, a citizen of the United States, residing in Elsmere, Delaware, have invented certain Improvements in Methods of Making Fiber Sheets, of which the following is a specification.

In the manufacture of the substance commonly known as vulcanized fiber, it is customary to form sheets of any desired thickness by pressing together a suitable number of relatively thin layers of paper one over the other, after they have been immersed in a bath of some material which parchments or gelatinizes their substance, it being usually customary to wind and compress upon a heated drum a suitable number of layers of the treated paper, and after the removal of the sheet thus formed, subjecting it to a treatment whereby all traces of the chemical with which it was treated are removed. In order to strip the laminated cylindrical body of treated paper from the roll, it is cut in a line substantially parallel with its axis and spread out flat, being thereafter soaked in water to permit of the removal and recovery of the chemical which it still contains, and finally dried. During the washing and drying process, a large proportion of the thick sheets formed are found to split to a greater or less degree, so that it is a common occurrence for sheets of one to two inches thickness to be rendered practically valueless by a separation of their layers, which begins at the edges and extends into and through the body for a greater or less distance.

One object of my invention, therefore, is to provide a method of treatment whereby this splitting or separation of the laminations of thick vulcanized fiber sheets during their manufacture shall be effectually prevented.

In carrying out my invention, a sheet of the desired thickness is formed by the superposition of any suitable number of layers of paper, fabric or the like immediately after it has been subjected to a so-called vulcanizing bath, such as a solution of hydrochloric acid and chlorid of zinc, the various layers being forced into intimate contact and subjected to heat. Thereafter, each laminated or composite sheet of the fiber is subjected, either immediately or at the end of any desired time, to one or more washing baths,

being preferably first immersed in a tank of cold water for a time depending upon its thickness, and thereafter removed to a tank of heated water. At any desired time during this washing step, and preferably just after it has been subjected to the washing in cold water, I bevel the edges of the sheet, that is, I cut them preferably at an angle of forty-five degrees to the plane of the sheet, both at the ends and at the sides thereof. Thereafter, the sheet is subjected to the washing or soaking out treatment in hot water and at the proper time, depending upon its thickness, is dried in the customary manner. As a result of this beveling of the edges of the treated sheets after they have been initially formed and before they are dry, I have found that the splitting or separation of the layers, even of the thickest sheets made, is effectually prevented.

While the cuts constituting this beveling are preferably made at an angle of forty-five degrees to the plane of the sheet, this angle may be varied in either direction, without departing from my invention, although I have found that when the sheets are left with their edges perpendicular to their planes, a splitting or separation occurs in a great majority of cases.

While I preferably bevel the edges just before the sheets are subjected to "soaking out" in hot water, since at this time they are most easily cut, it is obvious that the beveling may be done at any stage in the manufacture of the sheets after their formation and before drying, without departing from my invention.

I claim:—

1. The method which consists in the formation of a laminated sheet of parchmentized material; washing said sheet to remove the chemicals therein; and thereafter drying the sheet, the edges of said sheet being beveled at some time between its formation and the drying operation.

2. The method which consists in superposing a series of layers of parchmentized paper to form a laminated sheet; washing said sheet to remove the chemicals therefrom; beveling the edges of the sheet; and thereafter drying the sheet.

3. The method which consists in forming a laminated sheet of parchmentized fibrous material; subjecting said sheet to a plurality of washing operations to remove the

75

80

85

90

95

100

105

110

chemicals therefrom; beveling the edges of the sheet between two of the washing operations; and thereafter drying the sheet.

4. The method which consists in chemically treating vegetable fiber in sheet form to vulcanize the same; forming a sheet from a series of layers of said chemically treated material; washing said sheet to remove the chemicals therefrom; beveling the edges of the sheet; and thereafter drying the sheet.

5. The method which consists in forming a cylinder of layers of parchmentized paper; cutting said cylinder parallel with its axis to form a laminated sheet; washing said sheet to remove the chemicals therefrom; beveling the edges of the sheet; and drying the sheet.

6. The method which consists in forming a laminated sheet of a series of layers of paper which have been subjected to a bath containing chlorid of zinc; washing said lami-

nated sheet to remove the chlorid of zinc; beveling the edges of the sheet; and drying the sheet.

7. The method which consists in forming 25 a laminated sheet of parchmentized paper; washing said sheet in cold water; beveling the edges of the sheet; washing the sheet in hot water; and drying the sheet.

8. The method which consists in forming 30 a laminated parchmentized sheet; beveling the edges of the sheet while it is in a moist condition as a result of its formative treatment; and drying the sheet.

In testimony whereof, I have signed my 35 name to this specification, in the presence of two subscribing witnesses.

LEWIS N. JONES.

Witnesses:

WILLIAM E. BRADLEY,  
Wm. A. BARR.